

May 24, 1932.

W. MENDEL

1,860,314

TEXTILE FABRIC

Filed May 3, 1930



INVENTOR:

WILLIAM MENDEL,

*By Arthur E. Lang  
Attorney.*

## UNITED STATES PATENT OFFICE

WILLIAM MENDEL, OF BEVERLY, NEW JERSEY, ASSIGNOR TO NEIDICH VISCOSA CORPORATION, OF BURLINGTON, NEW JERSEY, A CORPORATION OF DELAWARE

## TEXTILE FABRIC

Application filed May 3, 1930. Serial No. 449,390.

My invention is particularly applicable to fabrics such as braids and ribbons designed and adapted for forming and decorating hat crowns, but is applicable to fabrics formed by ordinary cross weaving operations and to fabrics which are knit in either flat or tubular form; the essential feature of my invention being the inclusion in the pattern of a textile fabric of filaments which are respectively insoluble and soluble; the latter being removable by dissolving them after the fabric is formed and with the effect of modifying the pattern of the fabric by the dissolution of the soluble filaments. For instance, filaments of gelatinous materials, soluble in water, may be used in conjunction with yarns of ordinary textile fibers, to facilitate the formation of a pattern of the latter, and thereafter be dissolved from the fabric by merely dipping it in water. However, as water has at least a temporary softening effect upon most ordinary textile fibers, I prefer to employ filaments which are insoluble in water but soluble in other fluid which has no deleterious effect upon the other elements of the fabric. For instance, the soluble filaments may be formed of artificial cellulosic material such as cellulose nitrate or cellulose acetate, the latter being soluble in ethyl acetate or a mixture of alcohol and ether, and cellulose nitrate being soluble in acetone.

My invention includes the various novel features of construction, arrangement, and procedure hereinafter more definitely specified.

In said drawing; the figure is a face view of a textile fabric formed on a braiding machine and including soluble warp elements primarily so placed in the selvages of the fabric as to hold the weft threads in the desired pattern position until the fabric is finished. Said soluble warp elements have been dissolved from the lower portion of said fabric.

Referring to the form of my invention shown in the figure, the fabric 1 includes four distinct sets of weft filaments, respectively indicated at 2, 3, 4, and 5, preferably of a somewhat stiff and resilient character

such as may be formed of viscose, and four warp filaments respectively indicated at 7, 8, 9, and 10, formed of soluble material, for instance, cellulose acetate.

In the pattern shown in the figure, the weft filaments 2 and 3 are interlooped at the left hand edge of their extent in the fabric with the right hand edge of the extent of the filaments 4 in the fabric. Said filaments 2 and 3 are interlooped at the right hand edge of their extent in the fabric with the left hand edge of the extent of the filaments 5 in the fabric. Said soluble filament 7 forms a guide around which the weft filaments 3 and 4 are interlooped. Said soluble filament 8 forms a guide around which the weft filaments 3 and 5 are interlooped. Said soluble filament 9 forms a guide upon which the weft filaments 4 are decussated. Said soluble filament 10 forms a guide upon which the weft filaments 5 are decussated.

When thus formed, the insoluble filaments aforesaid take a permanent set in a pattern position determined by the presence of said soluble filaments 7, 8, 9, and 10 but, thereafter, said soluble filaments may be removed as indicated at the lower portion of the figure, without permitting the fabric to be thereafter distorted, and with the effect of imparting a lighter and more graceful appearance to the fabric than when the soluble threads were included therein.

It is to be understood that the fabrics chosen for illustration are merely typical embodiments of my invention which may be otherwise utilized.

Therefore, I do not desire to limit myself to the precise details of construction and arrangement herein set forth, as it is obvious that various modifications may be made therein without departing from the essential features of my invention, as defined in the appended claims.

I claim:

1. A braided textile fabric including a soluble filament with insoluble filaments; the soluble filament constituting a warp element of the fabric; the insoluble filaments including distinct groups interlooped upon said soluble filament as a guide. 95 100

2. A braided textile fabric formed entirely of artificial cellulosic material, but of different kinds, respectively soluble and insoluble in a given solvent; said soluble filaments forming guides for the fabrication of the insoluble filaments, which are interlooped thereon. 70
3. The process of forming a textile fabric wholly of artificial cellulosic filaments, but of different kinds, respectively soluble and insoluble in a given solvent, including interlooping the insoluble filaments upon the soluble filaments as guides, and subsequently dissolving the soluble filaments from the fabric. 75
4. The process of forming a braided textile fabric including artificial cellulosic filaments of different kinds, respectively soluble and insoluble in a given solvent, including interlooping the insoluble filaments upon the soluble filaments as guides, and subsequently dissolving the soluble filaments from the fabric. 80
5. A textile fabric including an insoluble filament pattern formed on a soluble filament frame extending within the fabric; said fabric including insoluble filaments permanently inseparably connecting regions thereof upon opposite sides of said frame. 85
6. A fabric as in claim 5; wherein the pattern is formed by insoluble filaments in decussated relation. 90
7. A fabric as in claim 5; wherein the frame is formed of artificial cellulosic material. 95
8. A fabric as in claim 5; wherein the pattern is formed by insoluble filaments in decussated relation on a frame of artificial cellulosic material. 100
9. A fabric as in claim 5; wherein the soluble filament frame includes a warp element in the fabric. 105
10. A fabric as in claim 5; wherein the soluble filament frame includes only warp elements in the fabric. 110
11. A textile fabric including an insoluble filament pattern formed on a soluble filament frame extending within the fabric wherein the pattern includes distinct groups of insoluble filaments interlooped upon the soluble frame. 115
12. The process of forming a textile fabric, including the formation of an insoluble filament pattern on a soluble filament warp frame, extending within the fabric, said fabric including insoluble filaments permanently inseparably connecting regions thereof upon opposite sides of said frame and thereafter dissolving out the frame. 120
13. The process of forming a textile fabric, including the formation of an insoluble artificial cellulosic filament pattern on a soluble artificial cellulosic warp frame, extending within the fabric, said fabric including insoluble filaments permanently inseparably connecting regions thereof upon 125
- In testimony whereof, I have hereunto signed my name at Burlington, New Jersey, this 29th day of April, 1930.
- WILLIAM MENDEL. 130